



US008409773B2

(12) **United States Patent**  
**Wu et al.**

(10) **Patent No.:** **US 8,409,773 B2**  
(45) **Date of Patent:** **Apr. 2, 2013**

(54) **EPOXY CARBOXYL RESIN MIXTURE HOLE BLOCKING LAYER PHOTOCODUCTORS**

(75) Inventors: **Jin Wu**, Webster, NY (US); **Marc J Livecchi**, Rochester, NY (US); **Robert W Hedrick**, Spencerport, NY (US); **John J. Wilbert**, Macedon, NY (US)

(73) Assignee: **Xerox Corporation**, Norwalk, CT (US)

(\*) Notice: Subject to any disclaimer, the term of this patent is extended or adjusted under 35 U.S.C. 154(b) by 589 days.

(21) Appl. No.: **12/394,343**

(22) Filed: **Feb. 27, 2009**

(65) **Prior Publication Data**

US 2010/0221651 A1 Sep. 2, 2010

(51) **Int. Cl.**

**G03G 15/00** (2006.01)

(52) **U.S. Cl.** ..... **430/58.8**; 430/56; 430/69; 430/58.05; 430/59.4

(58) **Field of Classification Search** ..... 430/109.3, 430/60, 58.5, 108.11, 58.8, 58.05, 59.4

See application file for complete search history.

(56) **References Cited**

U.S. PATENT DOCUMENTS

|                   |         |                                 |
|-------------------|---------|---------------------------------|
| 5,385,796 A       | 1/1995  | Spiewak et al.                  |
| 5,449,573 A       | 9/1995  | Aoki et al.                     |
| 5,928,824 A       | 7/1999  | Obinata et al.                  |
| 6,015,645 A       | 1/2000  | Murti et al.                    |
| 6,156,468 A       | 12/2000 | Wehelie et al.                  |
| 6,177,219 B1      | 1/2001  | Yuh et al.                      |
| 6,214,502 B1 *    | 4/2001  | Srinivasan et al. .... 430/58.4 |
| 6,255,027 B1      | 7/2001  | Wehelie et al.                  |
| 6,913,863 B2      | 7/2005  | Wu et al.                       |
| 7,037,631 B2      | 5/2006  | Wu et al.                       |
| 7,312,007 B2      | 12/2007 | Lin et al.                      |
| 7,485,398 B2      | 2/2009  | Wu et al.                       |
| 2005/0158640 A1 * | 7/2005  | Chambers et al. .... 430/60     |
| 2006/0105254 A1   | 5/2006  | Wu et al.                       |
| 2006/0204872 A1   | 9/2006  | Tong et al.                     |

|                   |         |                                 |
|-------------------|---------|---------------------------------|
| 2007/0049677 A1 * | 3/2007  | Wu et al. .... 524/430          |
| 2007/0243476 A1   | 10/2007 | Lin et al.                      |
| 2007/0298341 A1   | 12/2007 | Wu et al.                       |
| 2008/008947 A1    | 1/2008  | Wu                              |
| 2008/008951 A1 *  | 1/2008  | Wu et al. .... 430/58.8         |
| 2008/0032219 A1   | 2/2008  | Lin et al.                      |
| 2008/0153023 A1 * | 6/2008  | Yamazaki et al. .... 430/108.11 |
| 2008/0220350 A1   | 9/2008  | Wu et al.                       |
| 2008/0241721 A1 * | 10/2008 | Yuh et al. .... 430/58.8        |
| 2008/0311497 A1   | 12/2008 | Wu et al.                       |
| 2009/0035673 A1   | 2/2009  | Wu                              |
| 2009/0035674 A1   | 2/2009  | Wu                              |
| 2009/0035675 A1   | 2/2009  | Wu                              |
| 2009/0035676 A1   | 2/2009  | Wu                              |
| 2009/0047592 A1 * | 2/2009  | Okamoto et al. .... 430/109.3   |
| 2009/0245867 A1 * | 10/2009 | Wada et al. .... 399/159        |
| 2010/0221649 A1   | 9/2010  | Wu et al.                       |

FOREIGN PATENT DOCUMENTS

|    |              |           |
|----|--------------|-----------|
| EP | 1 818 726 A2 | 8/2007    |
| JP | 2007334335 A | * 12/2007 |

OTHER PUBLICATIONS

Sep. 6, 2010 European Search Report issued in EP 10 15 3961.  
Jin Wu et al., U.S. Application No. on Boron Containing Hole Blocking Layer Photoconductor, filed concurrently herewith.  
Jin Wu, U.S. Appl. No. 11/848,439 on Boron Containing Photoconductors, filed May 30, 2008.  
Jin Wu et al., U.S. Appl. No. 12/164,338 on Phenolic Resin Hole Blocking Layer Photoconductors, filed May 30, 2008.  
Jin Wu, U.S. Appl. No. 12/129,948 on Aminosilane and a Self Crosslinking Acrylic Resin Hole Blocking Layer Photoconductors, filed May 30, 2008.  
Jin Wu, U.S. Appl. No. 12/059,536 on Aminosilane and a Carbazole Hole Blocking Layer Photoconductors, filed Mar. 31, 2008.

\* cited by examiner

*Primary Examiner* — Mark F Huff

*Assistant Examiner* — Rashid Alam

(74) *Attorney, Agent, or Firm* — Eugene O. Palazzo

(57) **ABSTRACT**

A photoconductor that includes, for example, a substrate; an undercoat layer thereover wherein the undercoat layer contains a metal oxide, and a mixture of an epoxy resin and a carboxyl resin; a photogenerating layer; and at least one charge transport layer.

**25 Claims, No Drawings**

# EPOXY CARBOXYL RESIN MIXTURE HOLE BLOCKING LAYER PHOTOCONDUCTORS

## CROSS REFERENCE TO RELATED APPLICATIONS

U.S. application Ser. No. 12/394,178, U.S. Publication No. 20100221649, filed Feb. 27, 2009 on Boron Containing Hole Blocking Layer Photoconductor, the disclosure of which is totally incorporated herein by reference, illustrates a photoconductor comprising a substrate, a ground plane layer, an undercoat layer thereover wherein the undercoat layer comprises an aminosilane and a boron compound; a photogenerating layer, and a charge transport layer.

Illustrated in U.S. application Ser. No. 11/831,440, U.S. Publication 20090035673, now U.S. Pat. No. 7,871,748, filed Jul. 31, 2007, entitled Iron Containing Hole Blocking Layer Containing Photoconductors, the disclosure of which is totally incorporated herein by reference, is a photoconductor comprising a substrate; an undercoat layer thereover wherein the undercoat layer comprises a metal oxide, and an iron containing compound; a photogenerating layer; and at least one charge transport layer.

Illustrated in U.S. application Ser. No. 11/831,453, U.S. Publication 20090035674, now U.S. Pat. No. 7,670,737, filed Jul. 31, 2007, entitled UV Absorbing Hole Blocking Layer Containing Photoconductors, the disclosure of which is totally incorporated herein by reference, is a photoconductor comprising a substrate; an undercoat layer thereover wherein the undercoat layer comprises a metal oxide, and an ultraviolet light absorber component; a photogenerating layer; and at least one charge transport layer.

Illustrated in U.S. application Ser. No. 11/831,476, U.S. Publication 20090035676, now U.S. Pat. No. 7,851,115, filed Jul. 31, 2007, entitled Iodonium Hole Blocking Layer Photoconductor, the disclosure of which is totally incorporated herein by reference, is a photoconductor comprising a substrate; an undercoat layer thereover wherein the undercoat layer comprises a metal oxide and an iodonium containing compound; a photogenerating layer; and at least one charge transport layer.

Illustrated in U.S. application Ser. No. 11/831,469, U.S. Publication No. 20090035675, now U.S. Pat. No. 7,867,676, filed Jul. 11, 2007, entitled Copper Containing Hole Blocking Layer Photoconductors, the disclosure of which is totally incorporated herein by reference, is a photoconductor comprising a substrate; an undercoat layer thereover wherein the undercoat layer comprises a metal oxide, and a copper containing compound; a photogenerating layer; and at least one charge transport layer.

Illustrated in U.S. application Ser. No. 11/211,757, U.S. Publication No. 20070049677, now U.S. Pat. No. 7,544,452, filed Aug. 26, 2005, entitled Thick Electrophotographic Imaging Member Undercoat Layers, the disclosure of which is totally incorporated herein by reference, are binders containing metal oxide nanoparticles and a co-resin of phenolic resin and aminoplast resin, and an electrophotographic imaging member undercoat layer containing the binders.

Illustrated in U.S. application Ser. No. 10/942,277, U.S. Publication No. 20060057480, U.S. Pat. No. 7,312,007, filed Sep. 16, 2004, entitled Photoconductive Imaging Members, the disclosure of which is totally incorporated herein by reference, is a photoconductive member containing a hole blocking layer, a photogenerating layer, and a charge transport layer, and wherein the hole blocking layer contains a metallic component like a titanium oxide and a polymeric binder.

Illustrated in U.S. application Ser. No. 11/764,489, U.S. Publication 20080311497, now U.S. Pat. No. 7,846,628, filed Jun. 18, 2007, entitled Hole Blocking Layer Containing Photoconductors, the disclosure of which is totally incorporated herein by reference, is a photoconductor comprising a substrate; an undercoat layer thereover wherein the undercoat layer comprises a metal oxide, an electron donor and an electron acceptor charge transfer complex; a photogenerating layer; and at least one charge transport layer.

Illustrated in U.S. application Ser. No. 11/403,981, U.S. Publication 20070243476, now U.S. Pat. No. 7,604,914, filed Apr. 13, 2006, entitled Imaging Members, the disclosure of which is totally incorporated herein by reference, is an electrophotographic imaging member, comprising a substrate, an undercoat layer disposed on the substrate, wherein the undercoat layer comprises a polyol resin, an aminoplast resin, and a metal oxide dispersed therein; and at least one imaging layer formed on the undercoat layer, and wherein the polyol resin is, for example, selected from the group consisting of acrylic polyols, polyglycols, polyglycerols, and mixtures thereof.

Illustrated in U.S. patent application Ser. No. 11/481,642, U.S. Publication 20080008947, now U.S. Pat. No. 7,732,112, filed Jul. 6, 2006, the disclosure of which is totally incorporated by reference herein, is an imaging member including a substrate; a charge generation layer positioned on the substrate; at least one charge transport layer positioned on the charge generation layer; and an undercoat or hole blocking layer positioned on the substrate on a side opposite the charge generation layer, the undercoat layer comprising a binder component and a metallic component comprising a metal thiocyanate and metal oxide.

Disclosed in U.S. application Ser. No. 11/496,790, U.S. Publication 20080032219, now U.S. Pat. No. 7,560,208, filed Aug. 1, 2006, the disclosure of which is totally incorporated herein by reference, is a photoconductor member comprising a substrate; an undercoat layer thereover wherein the undercoat layer comprises a polyol resin, an aminoplast resin, a polyester adhesion component and a metal oxide; and at least one imaging layer formed on the undercoat layer.

Disclosed in U.S. application Ser. No. 11/714,600, U.S. Publication No. 20080220350, now U.S. Pat. No. 7,579,126, filed Mar. 6, 2007, the disclosure of which is totally incorporated herein by reference, is a photoconductor comprising a substrate; an undercoat layer thereover wherein the undercoat layer comprises an electroconducting component dispersed in a rapid curing polymer matrix; a photogenerating layer, and at least one charge transport layer.

The appropriate components and processes, number and sequence of the layers, component and component amounts in each layer, and the thicknesses of each layer of the above copending applications, may be selected for the present disclosure photoconductors in embodiments thereof.

## BACKGROUND

There are disclosed herein hole blocking layers, and more specifically, photoconductors containing a hole blocking layer or undercoat layer (UCL) comprised, for example, of a metal oxide, and a mixture of an epoxy resin and a carboxyl resin, and which layer can be situated between the supporting substrate and the photogenerating layer. More specifically, there are disclosed herein an epoxy and carboxyl resin mixture containing undercoat or hole blocking layers which further include some of the components as illustrated in the copending applications referred to herein, such as a metal oxide like a titanium dioxide.

In embodiments, photoconductors comprised of the disclosed hole blocking or undercoat layer enables, for example, the minimization or substantial elimination of undesirable ghosting on developed images, such as xerographic images, including excellent ghosting at various relative humidities; excellent cyclic and stable electrical properties; minimal charge deficient spots (CDS); and compatibility with the photogenerating and charge transport resin binders, such as polycarbonates. Charge blocking layer and hole blocking layer are generally used interchangeably with the phrase "undercoat layer".

The need for excellent print quality in xerographic systems is of value, especially with the advent of color. Common print quality issues can be dependent on the components of the undercoat layer (UCL). In certain situations, a thicker undercoat is desirable, but the thickness of the material used for the undercoat layer may be limited by, in some instances, the inefficient transport of the photojected electrons from the generator layer to the substrate. When the undercoat layer is too thin, then incomplete coverage of the substrate may sometimes result due to wetting problems on localized unclean substrate surface areas. The incomplete coverage produces pin holes which can, in turn, produce print defects such as charge deficient spots (CDS) and bias charge roll (BCR) leakage breakdown. Other problems include "ghosting" resulting from, it is believed, the accumulation of charge somewhere in the photoreceptor. Removing trapped electrons and holes residing in the imaging members is a factor to preventing ghosting. During the exposure and development stages of xerographic cycles, the trapped electrons are mainly at or near the interface between the photogenerating layer (CGL) and the undercoat layer (UCL), and holes are present mainly at or near the interface between the photogenerating layer and the charge transport layer (CTL). The trapped charges can migrate according to the electric field during the transfer stage where the electrons can move from the interface of CGL/UCL to CTL/CGL, or the holes from CTL/CGL to CGL/UCL, and become deep traps that are no longer mobile. Consequently, when a sequential image is printed, the accumulated charge results in image density changes in the current printed image that reveals the previously printed image. Thus, there is a need to minimize or eliminate charge accumulation in photoreceptors without sacrificing the desired thickness of the undercoat layer, and a need for permitting the UCL to properly adhere to the other photoconductive layers, such as the photogenerating layer, for extended time periods, such as for example, about 2,000,000 simulated xerographic imaging cycles. Thus, conventional materials used for the undercoat or blocking layer possess a number of disadvantages resulting in adverse print quality characteristics, which disadvantages include, for example, ghosting, charge deficient spots, and bias charge roll leakage breakdown are problems that commonly occur. Ghosting, it is believed, results from the accumulation of charge in the photoconductor, therefore, when a sequential xerographic image is printed, the accumulated charge results in image density changes that reveals the previously printed image.

Thick undercoat layers are sometimes desirable for xerographic photoconductors as such layers permit photoconductor life extension and carbon fiber resistance. Furthermore, thicker undercoat layers permit the use of economical substrates in the photoreceptors. Examples of thick undercoat layers are disclosed in U.S. application Ser. No. 10/942,277, filed Sep. 16, 2004, U.S. Publication 20060057480, entitled Photoconductive Imaging Members, the entire disclosure of which is totally incorporated herein by reference. However, due primarily to insufficient electron conductivity in dry and

cold environments, the residual potential in conditions, such as 10 percent relative humidity and 70° F., can be high when the undercoat layer is thicker than about 15 microns, and moreover, the adhesion of the UCL may be poor, disadvantages avoided or minimized with the UCL of the present disclosure.

Also included within the scope of the present disclosure are methods of imaging and printing with the photoconductive devices illustrated herein. These methods generally involve 10 the formation of an electrostatic latent image on the imaging member, followed by developing the image with a toner composition comprised, for example, of a thermoplastic resin, colorant, such as pigment, charge additive, and surface additives, reference U.S. Pat. Nos. 4,560,635; 4,298,697 and 15 4,338,390, the disclosures of which are totally incorporated herein by reference, subsequently transferring the image to a suitable substrate, and permanently affixing the image thereto. In those environments wherein the device is to be used in a printing mode, the imaging method involves the 20 same operation with the exception that exposure can be accomplished with a laser device or image bar. More specifically, the imaging members, photoconductor drums, and flexible belts disclosed herein can be selected for the Xerox Corporation iGEN3® machines that generate with some versions over 100 copies per minute. Processes of imaging, especially xerographic imaging and printing, including digital, and/or high speed color printing, are thus encompassed by the present disclosure.

The photoconductors disclosed herein are, in embodiments, sensitive in the wavelength region of, for example, from about 400 to about 900 nanometers, and in particular from about 650 to about 850 nanometers, thus diode lasers can be selected as the light source.

## REFERENCES

Illustrated in U.S. Pat. No. 6,913,863 is a photoconductive imaging member comprised of an optional supporting substrate, a hole blocking layer thereover, a photogenerating layer, and a charge transport layer, and wherein the hole blocking layer is comprised of a metal oxide, a mixture of phenolic resins, and wherein at least one of the resins contains two hydroxy groups.

Illustrated in U.S. Pat. Nos. 6,255,027; 6,177,219, and 45 6,156,468, are, for example, photoreceptors containing a charge blocking layer of a plurality of light scattering particles dispersed in a binder, reference for example, Example I of U.S. Pat. No. 6,156,468, wherein there is illustrated a charge blocking layer of titanium dioxide dispersed in a specific linear phenolic binder of VARCUM®, available from OxyChem Company.

Illustrated in U.S. Pat. No. 6,015,645, is a photoconductive imaging member comprised of a supporting substrate, a hole blocking layer, an optional adhesive layer, a photogenerating layer, and a charge transport layer, and wherein the blocking layer is comprised of a polyhaloalkylstyrene.

Layered photoconductors have been described in numerous U.S. patents, such as U.S. Pat. No. 4,265,990.

In U.S. Pat. No. 4,921,769, there are illustrated photoconductive imaging members with blocking layers of certain polyurethanes.

Illustrated in U.S. Pat. No. 5,473,064, the disclosure of which is totally incorporated herein by reference, is a process for the preparation of hydroxygallium phthalocyanine Type V, essentially free of chlorine.

Illustrated in U.S. Pat. No. 5,521,306, the disclosure of which is totally incorporated herein by reference, is a process

for the preparation of Type V hydroxygallium phthalocyanine comprising the in situ formation of an alkoxy-bridged gallium phthalocyanine dimer, hydrolyzing the dimer to hydroxygallium phthalocyanine, and subsequently converting the hydroxygallium phthalocyanine product to Type V hydroxygallium phthalocyanine.

Illustrated in U.S. Pat. No. 5,482,811, the disclosure of which is totally incorporated herein by reference, is a process for the preparation of hydroxygallium phthalocyanine photo-generating pigments, which comprises hydrolyzing a gallium phthalocyanine precursor pigment by dissolving the hydroxygallium phthalocyanine in a strong acid, and then reprecipitating the resulting dissolved pigment in basic aqueous media; removing any ionic species formed by washing with water, concentrating the resulting aqueous slurry comprised of water and hydroxygallium phthalocyanine to a wet cake; removing water from said slurry by azeotropic distillation with an organic solvent, and subjecting said resulting pigment slurry to mixing with the addition of a second solvent to cause the formation of said hydroxygallium phthalocyanine polymorphs.

A number of photoconductors are disclosed in U.S. Pat. Nos. 5,489,496; 4,579,801; 4,518,669; 4,775,605; ; 5,641,599; 5,344,734; 5,721,080; and U.S. Pat. No. 5,017,449, the entire disclosures of which are totally incorporated herein by reference. Also, photoreceptors are disclosed in U.S. Pat. Nos. 6,200,716; 6,180,309; and U.S. Pat. No. 6,207,334, the entire disclosures of which are totally incorporated herein by reference.

A number of undercoat or charge blocking layers are disclosed in U.S. Pat. Nos. 4,464,450; 5,449,573; 5,385,796; and U.S. Pat. No. 5,928,824, the entire disclosures of which are totally incorporated herein by reference.

## SUMMARY

According to embodiments illustrated herein, there are provided photoconductors that enable acceptable print quality, and wherein ghosting is minimized or substantially eliminated in images printed in systems with high transfer current, and where charge deficient spots (CDS) resulting, for example, from the photogenerating layer, and causing printable defects is minimized, and more specifically, where the CDSs are low, such as from about 30 to about 90 percent lower as compared to a similar photoconductor with a known hole blocking layer.

Embodiments disclosed herein also include a photoconductor comprising a substrate, an undercoat layer as illustrated herein, disposed or deposited on the substrate, and a photogenerating layer and charge transport layer formed on the undercoat layer; a photoconductor comprised of a substrate, an undercoat layer disposed on the substrate, wherein the undercoat layer comprises a metal oxide like titanium dioxide, and a mixture of an epoxy resin and a carboxyl resin which primarily functions to inhibit ghosting characteristics for the photoconductor.

## DETAILED DESCRIPTION

Aspects of the present disclosure relate to a photoconductor comprising a substrate; an undercoat layer thereover wherein the undercoat layer comprises a metal oxide, and a mixture of an epoxy resin and a carboxyl resin; a photogenerating layer; and at least one charge transport layer; a photoconductor comprising a supporting substrate; an undercoat layer thereover comprised of a mixture of a metal oxide, and a mixture of an epoxy resin and a carboxyl resin; a photoge-

nerating layer; and a charge transport layer; a rigid or flexible photoconductor comprising in sequence a supporting substrate; a hole blocking layer comprised, for example, of a titanium oxide, and a mixture of an epoxy resin and a carboxyl resin; a photogenerating layer; and a charge transport layer; a photoconductive member or device comprising a substrate, the robust undercoat layer illustrated herein, and at least one imaging layer, such as a photogenerating layer and a charge transport layer or layers, formed on the undercoat layer; a photoconductor wherein the photogenerating layer is situated between the charge transport layer and the substrate, and which layer contains a resin binder; an electrophotographic imaging member which generally comprises at least a substrate layer, an undercoat layer, and where the undercoat layer is generally located between the substrate and deposited on the undercoat layer in sequence a photogenerating layer and a charge transport layer; a photoconductor comprising a substrate; an undercoat layer thereover wherein the undercoat layer comprises a metal oxide, and a mixture of the resins illustrated herein; a photogenerating layer; and at least one charge transport layer; a photoconductor comprising a substrate, an undercoat layer thereover comprised of a mixture of a metal oxide, an epoxy resin, and a carboxyl resin; a photogenerating layer; and a charge transport layer; and a rigid or flexible photoconductor comprising in sequence a supporting substrate; a resin mixture metal oxide hole blocking layer; a photogenerating layer; and at least one charge transport layer.

In embodiments, the undercoat layer metal oxide like  $TiO_2$  can be either surface treated or untreated. Surface treatments include, but are not limited to, mixing the metal oxide with aluminum laurate, alumina, zirconia, silica, silane, methicone, dimethicone, sodium metaphosphate, and the like, and mixtures thereof. Examples of  $TiO_2$  include MT-150W<sup>TM</sup> (surface treatment with sodium metaphosphate, available from Tayca Corporation), STR-60N<sup>TM</sup> (no surface treatment, available from Sakai Chemical Industry Co., Ltd.), FTL-100<sup>TM</sup> surface treatment, available from Ishihara Sangyo Laisha, Ltd., STR-60<sup>TM</sup> (surface treatment with  $Al_2O_3$ , available from Sakai Chemical Industry Co., Ltd.), TTO-55N<sup>TM</sup> (no surface treatment, available from Ishihara Sangyo Laisha, Ltd.), TTO-55A<sup>TM</sup> (surface treatment with  $Al_2O_3$ , available from Ishihara Sangyo Laisha, Ltd.), MT-150AW<sup>TM</sup> (no surface treatment, available from Tayca Corporation), MT-150A<sup>TM</sup> (no surface treatment, available from Tayca Corporation), MT-100S<sup>TM</sup> (surface treatment with aluminum laurate and alumina, available from Tayca Corporation), MT-100HD<sup>TM</sup> (surface treatment with zirconia and alumina, available from Tayca Corporation), MT-100SA<sup>TM</sup> (surface treatment with silica and alumina, available from Tayca Corporation), and the like.

Examples of metal oxides present in suitable amounts, such as for example, from about 5 to about 80 weight percent, and more specifically, from about 40 to about 70 weight percent, are titanium oxides and mixtures of metal oxides thereof. In embodiments, the metal oxide has a size diameter of from about 5 to about 300 nanometers, a powder resistance of from about  $1 \times 10^3$  to about  $6 \times 10^5$  ohm/cm when applied at a pressure of from about 50 to about 650 kilograms/cm<sup>2</sup>, and yet more specifically, the titanium oxide possesses a primary particle size diameter of from about 10 to about 25 nanometers, and more specifically, from about 12 to about 17, and yet more specifically, about 15 nanometers with an estimated aspect ratio of from about 4 to about 5, and is optionally surface treated with, for example, a component containing, for example, from about 1 to about 3 percent by weight of alkali metal, such as a sodium metaphosphate, a powder resistance of from about  $1 \times 10^4$  to about  $6 \times 10^4$  ohm/cm when

applied at a pressure of from about 650 to about 50 kilograms/cm<sup>2</sup>, MT-150W<sup>TM</sup>, and which titanium oxide is available from Tayca Corporation, and wherein the hole blocking layer is of a suitable thickness, such as a thickness of about from about 0.1 to about 15 microns, thereby avoiding or minimizing charge leakage. Metal oxide examples in addition to titanium are chromium, zinc, tin, copper, antimony, and the like, and more specifically, zinc oxide, tin oxide, aluminum oxide, silicone oxide, zirconium oxide, indium oxide, molybdenum oxide, and mixtures thereof.

#### NONLIMITING EXAMPLES OF RESIN MIXTURES

Specific nonlimiting examples of the epoxy resin are diglycidyl ether of bisphenol A, diglycidyl ether of bisphenol F resins and modified resins and blends thereof.

Specific diglycidyl ether of bisphenol A liquid epoxy resins include EPON<sup>TM</sup> 825 (175 to 180 weight per epoxide), 834 (230 to 280 weight per epoxide), 824 (192 to 204 weight per epoxide), 8280 (185 to 195 weight per epoxide), and 872 (625 to 725 weight per epoxide). Specific diglycidyl ether of bisphenol F liquid epoxy resins include EPON<sup>TM</sup> 862 (165 to 173 weight per epoxide), and 863 (165 to 174 weight per epoxide). Specific diglycidyl ether of bisphenol F and bisphenol A blend liquid epoxy resins include EPON<sup>TM</sup> 235 (177 to 182 weight per epoxide), all commercially available from HEXION Specialty Chemicals, Columbus, Ohio. These liquid epoxy resins can be further blended with alkyl glycidyl ether as in EPON<sup>TM</sup> 8132, cresyl glycidyl ether as in EPON<sup>TM</sup> 813, butyl glycidyl ether as in EPON<sup>TM</sup> 815C, castor oil glycidyl ether as in EPON<sup>TM</sup> 8131, and other glycidyl ethers, all commercially available from HEXION Specialty Chemicals, Columbus, Ohio.

Epoxy resins can also be in solutions in solvents, such as acetone, methyl ethyl ketone, methyl isobutyl ketone (MIBK), diacetone alcohol, isopropyl alcohol, n-butyl alcohol, n-butyl acetate, propylene glycol monomethyl ether, isobutyl alcohol, ethyl 3-ethoxypropionate, t-butyl acetate, propylene glycol mono(n-butyl)ether, ethylene glycol monobutyl ether, methyl n-amyl ketone, n-propyl alcohol, propylene glycol monomethyl ether acetate, dimethylformamide, cyclohexanone, toluene, aromatic 100, dipropylene glycol monomethyl ether, water, xylene, ethylene glycol monopropyl ether, and the like, and mixtures thereof.

Specific diglycidyl ether of bisphenol A solution epoxy resins include EPON<sup>TM</sup> 828-X-95 (193 to 204 weight per epoxide, 95 percent solids in xylene), 8521-MX-60 (750 to 850 weight per epoxide, 60 percent solids in ethylene glycol monobutyl ether/xylene), 1001-T-75 (450 to 550 weight per epoxide, 75 percent solids in toluene), 1004-O-65 (850 to 1,050 weight per epoxide, 65 percent solids in methyl n-amyl ketone), 1007-CT-55 (1,600 to 2,300 weight per epoxide, 55 percent solids in MIBK/toluene), and 1009-MV-40 (2,500 to 4,000 weight per epoxide, 40 percent solids in ethylene glycol monobutyl ether/dipropylene glycol monomethyl ether), all commercially available from HEXION Specialty Chemicals, Columbus, Ohio. These solution epoxy resins can be further blended with alkyl C12 to C14 glycidyl ether as in EPON<sup>TM</sup> CS 243, and p-tert-butyl phenyl glycidyl ether as in EPON<sup>TM</sup> CS 377, all commercially available from HEXION Specialty Chemicals, Columbus, Ohio.

Other epoxy resins that can be selected as part of the resin mixture hole blocking layer include tetraglycidyl ether of tetraphenol ethane resins such as EPON<sup>TM</sup> 1031 (195 to 230 weight per epoxide), epoxy phenolic novolac resins such as EPON<sup>TM</sup> 154 (176 to 181 weight per epoxide), epoxy bisphe-

nol A novolac resins such as EPON<sup>TM</sup> SU-2.5 (180 to 200 weight per epoxide), epoxy bisphenol F novolac resins such as EPON<sup>TM</sup> 160 (168 to 178 weight per epoxide), epoxy cresol novolac resins such as EPON<sup>TM</sup> 164 (200 to 240 weight per epoxide), epoxy polyacrylates such as EPON<sup>TM</sup> 8111 (140 weight per epoxide), elastomer modified epoxy resins such as EPON<sup>TM</sup> 58005 (325 to 375 weight per epoxide), hydrogenated diglycidyl ether of bisphenol A (cycloaliphatic glycidyl ether) resins such as EPONEX<sup>TM</sup> 1510 (210 to 220 weight per epoxide), and brominated epoxy resins such as EPON<sup>TM</sup> 1183 (625 to 725 weight per epoxide), all commercially available from HEXION Specialty Chemicals, Columbus, Ohio.

The epoxy resins possess, for example, a number average molecular weight of from about 50 to about 10,000, from about 200 to about 4,000, or from about 400 to about 1,000, and a weight average molecular weight of from about 60 to about 30,000, from about 250 to about 12,000, or from about 500 to about 3,000, present in an amount of from about 5 to about 90 weight percent, or from about 10 to about 40 weight percent of the total hole blocking layer solids.

Specific nonlimiting examples of the carboxyl resin are acrylic carboxyl resins. In embodiments, acrylic carboxyl resin examples include copolymers of acrylic acid and/or methacrylic acid, and/or their derivatives including acrylic and methacrylic esters and components containing nitrile and amide groups, and other optional monomers. The acrylic esters can be selected from, for example, the group consisting of n-alkyl acrylates wherein alkyl contains, in embodiments, from 1 to about 25 carbon atoms, such as methyl, ethyl, propyl, butyl, pentyl, hexyl, heptyl, octyl, nonyl, decyl, dodecyl, tetradecyl, or hexadecyl acrylate; secondary and branched-chain alkyl acrylates such as isopropyl, isobutyl, sec-butyl, 2-ethylhexyl, or 2-ethylbutyl acrylate; olefinic acrylates such as allyl, 2-methylallyl, furfuryl, or 2-but enyl acrylate; aminoalkyl acrylates such as 2-(dimethylamino)ethyl, 2-(diethylamino)ethyl, 2-(dibutylamino)ethyl, or 3-(diethylamino)propyl acrylate; ether acrylates such as 2-methoxyethyl, 2-ethoxyethyl, tetrahydrofurfuryl, or 2-butoxyethyl acrylate; cycloalkyl acrylates such as cyclohexyl, 4-methylcyclohexyl, or 3,3,5-trimethylcyclohexyl acrylate; halogenated alkyl acrylates such as 2-bromoethyl, 2-chloroethyl, or 2,3-dibromopropyl acrylate; glycol acrylates and diacrylates such as ethylene glycol, propylene glycol, 1,3-propanediol, 1,4-butanediol, diethylene glycol, 1,5-pentanediol, triethylene glycol, dipropylene glycol, 2,5-hexanediol, 2,2-diethyl-1,3-propanediol, 2-ethyl-1,3-hexanediol, or 1,10-decanediol acrylate, and diacrylate. Examples of methacrylic esters can be selected from, for example, the group consisting of alkyl methacrylates such as methyl, ethyl, propyl, isopropyl, n-butyl, isobutyl, sec-butyl, t-butyl, n-hexyl, n-octyl, isooctyl, 2-ethylhexyl, n-decyl, or tetradecyl methacrylate; unsaturated alkyl methacrylates such as vinyl, allyl, oleyl, or 2-propynyl methacrylate; cycloalkyl methacrylates such as cyclohexyl, 1-methylcyclohexyl, 3-vinylcyclohexyl, 3,3,5-trimethylcyclohexyl, bornyl, isobornyl, or cyclopenta-2,4-dienyl methacrylate; aryl methacrylates such as phenyl, benzyl, or nonylphenyl methacrylate; hydroxyalkyl methacrylates such as 2-hydroxyethyl, 2-hydroxypropyl, 3-hydroxypropyl, or 3,4-dihydroxybutyl methacrylate; ether methacrylates such as methoxymethyl, ethoxymethyl, 2-ethoxyethoxymethyl, allyloxymethyl, benzoyloxymethyl, cyclohexyloxymethyl, 1-ethoxyethyl, 2-ethoxyethyl, 2-butoxyethyl, 1-methyl-(2-vinyl)oxethyl, methoxymethoxyethyl, methoxyethoxyethyl, vinyloxyethoxyethyl, 1-butoxypropyl, 1-ethoxybutyl, tetrahydrofurfuryl, or furfuryl methacrylate; oxiranyl methacrylates such

as glycidyl, 2,3-epoxybutyl, 3,4-epoxybutyl, 2,3-epoxycyclohexyl, or 10,11-epoxyundecyl methacrylate; aminoalkyl methacrylates such as 2-dimethylaminoethyl, 2-diethylaminoethyl, 2-t-octylaminoethyl, N,N-dibutylaminoethyl, 3-diethylaminopropyl, 7-amino-3,4-dimethyoctyl, N-methylformamidoethyl, or 2-ureidoethyl methacrylate; glycol dimethacrylates such as methylene, ethylene glycol, 1,2-propanediol, 1,3-butanediol, 1,4-butanediol, 2,5-dimethyl-1,6-hexanediol, 1,10-decanediol, diethylene glycol, or triethylene glycol dimethacrylate; trimethacrylates such as trimethylolpropane trimethacrylate; carbonyl-containing methacrylates such as carboxymethyl, 2-carboxyethyl, acetyl, oxazolidinylethyl, N-(2-methacryloyloxyethyl)-2-pyrrolidinone, N-methacryloyl-2-pyrrolidinone, N-(methacryloyloxy)formamide, N-methacryloylmorpholine, or tris(2-methacryloyloxyethyl)amine methacrylate; other nitrogen-containing methacrylates such as 2-methacryloyloxyethylmethyl cyanamide, methacryloyloxyethyltrimethylammonium chloride, N-(methacryloyloxy-ethyl)diisobutylketimine, cyanomethyl, or 2-cyanoethyl methacrylate; halogenated alkyl methacrylates such as chloromethyl, 1,3-dichloro-2-propyl, 4-bromophenyl, 2-bromoethyl, 2,3-dibromopropyl, or 2-iodoethyl methacrylate; sulfur-containing methacrylates such as methylthiol, butylthiol, ethylsulfonylethyl, ethylsulfanylethyl, thiocyanatomethyl, 4-thiocyanatobutyl, methylsulfanyl methyl, 2-dodecylthioethyl methacrylate, or bis(methacryloyloxyethyl)sulfide; phosphorous-boron-silicon-containing methacrylates such as 2-(ethylenephosphino)propyl, dimethylphosphinomethyl, dimethylphosphonoethyl, diethylphosphatoethyl, 2-(dimethylphosphato)propyl, 2-(dimethylphosphono)ethyl methacrylate, diethyl methacryloylphosphonate, dipropyl methacryloyl phosphate, diethyl methacryloyl phosphite, 2-methacryloyloxyethyl diethyl phosphite, 2,3-butylene methacryloyloxyethyl borate, or methylidiethoxymethacryloyloxyethoxysilane. Methacrylic amides and nitriles can be selected from the group consisting of at least one of N-methylmethacrylamide, N-isopropylmethacrylamide, N-phenylmethacrylamide, N-(2-hydroxyethyl)methacrylamide, 1-methacryloylamido-2-methyl-2-propanol, 4-methacryloylamido-4-methyl-2-pentanol, N-(methoxymethyl)methacrylamide, N-(dimethylaminoethyl)methacrylamide, N-(3-dimethylaminopropyl)methacrylamide, N-acetyl methacrylamide, N-methacryloylmaleimic acid, methacryloylamido acetonitrile, N-(2-cyanoethyl) methacrylamide, 1-methacryloylurea, N-phenyl-N-phenylethylmethacrylamide, N-(3-dibutylaminopropyl)methacrylamide, N,N-diethylmethacrylamide, N-(2-cyanoethyl)-N-methylmethacrylamide, N,N-bis(2-diethylaminoethyl)methacrylamide, N-methyl-N-phenylmethacrylamide, N,N'-methylenebismethacrylamide, N,N'-ethylenebismethacrylamide, or N-(diethylphosphono)methacrylamide. Further optional monomer examples are styrene, acrolein, acrylic anhydride, acrylonitrile, acryloyl chloride, methacrolein, methacrylonitrile, methacrylic anhydride, methacrylic acetic anhydride, methacryloyl chloride, methacryloyl bromide, itaconic acid, butadiene, vinyl chloride, vinylidene chloride, or vinyl acetate.

Specific acrylic carboxyl resin examples include PARALOID® AT-85 ( $T_g=9^\circ C$ ., acid number=65, 55.5 percent solid in aromatic 150/butyl cellusolve=87/13), PARALOID® AT-81 ( $T_g=40^\circ C$ ., acid number=65, 55.5 percent solid in aromatic 150/butyl cellusolve=87/13), PARALOID® AT-76 ( $T_g=25^\circ C$ ., acid number=38, 41 percent solid in aromatic 150/butyl cellusolve=75/25), PARALOID® AT-148 ( $T_g=9^\circ C$ ., acid number=65, 55 percent solid in butyl cellusolve), PARALOID® AT-147 ( $T_g=40^\circ C$ ., acid number=65, 55 per-

cent solid in butyl cellusolve), and PARALOID® AT-9LO ( $T_g=30^\circ C$ ., acid number=35, 45 percent solid in aromatic 150/butyl cellusolve=90/10), all commercially available from Rohm and Haas.

5 The number average molecular weight of the carboxyl resin is, for example, from about 400 to about 50,000, or from about 1,000 to about 10,000. The weight average molecular weight of the carboxyl resin is from about 500 to about 100,000, or from about 1,500 to about 20,000. The carboxyl 10 resin is present in an amount of from about 5 to about 90 weight percent, or from about 10 to about 40 weight percent of the total hole blocking layer solids.

The hole blocking layer further comprises an acid catalyst or a base catalyst to accelerate the crosslinking reactions 15 between the two resins. Non-limiting examples of the acid catalyst include oxalic acid, maleic acid, carboxylic acid, ascorbic acid, malonic acid, succinic acid, tartaric acid, citric acid, p-toluenesulfonic acid, methanesulfonic acid, and the like, and mixtures thereof. A typical concentration of the acid 20 catalyst is from about 0.1 to about 5 weight percent or from about 0.5 to about 2 weight percent based on the total weight of the two resins. Non-limiting examples of the base catalyst are amines, such as triethyl amine, diethylenetriamine, triethylenetetramine, isphoronediamine, bis-p-aminocyclohexyl 25 methane, 1,2-diaminocyclohexane, diaminodiphenylmethane, and the like, and the mixtures thereof. A typical concentration of the base catalyst is from about 0.1 to about 10 weight percent, or from about 0.5 to about 4 weight percent based on the total weight of the two resins.

30 Examples of amounts of the resin mixture that is present in the hole blocking layer can vary, and be, for example, from about 10 to about 95 weight percent, from about 20 to about 60 weight percent, and more specifically, from about 30 to about 40 weight percent, based on the weight percentages of 35 the components contained in the hole blocking layer.

The weight ratio of the epoxy resin and the carboxyl resin of the resin mixture is from about 10/90 to about 90/10, from about 20/80 to about 80/20, or from about 40/60 to about 60/40.

40 The hole blocking layer can, in embodiments, be prepared by a number of known methods, the process parameters being dependent, for example, on the photoconductor member desired. The hole blocking layer can be coated as a dispersion onto a substrate by the use of a spray coater, dip coater, extrusion coater, roller coater, wire-bar coater, slot coater, doctor blade coater, gravure coater, and the like, and dried at from about 40°C. to about 240°C., or from about 140°C. to about 200°C. for a suitable period of time, such as from about 1 minute to about 10 hours, or from about 10 to about 60 minutes, under stationary conditions or in an air flow. The coating can be accomplished to provide a final coating thickness of from about 0.1 to about 30 microns, from about 1 to about 20 microns, or from about 5 to about 15 microns after drying.

55 In embodiments, the hole blocking layer may contain various colorants such as organic pigments and organic dyes, including, but not limited to, azo pigments, quinoline pigments, perylene pigments, indigo pigments, thioindigo pigments, bisbenzimidazole pigments, phthalocyanine pigments, quinacridone pigments, quinoline pigments, lake pigments, azo lake pigments, anthraquinone pigments, oxazine pigments, dioxazine pigments, triphenylmethane pigments, azulene dyes, squalium dyes, pyrilium dyes, triallylmethane dyes, xanthene dyes, thiazine dyes, and cyanine dyes. In various embodiments, the hole blocking layer 60 may include inorganic materials, such as amorphous silicon, amorphous selenium, tellurium, a selenium-tellurium alloy,

## 11

cadmium sulfide, antimony sulfide, titanium oxide, tin oxide, zinc oxide, and zinc sulfide, and mixtures thereof. The colorant can be selected in various suitable amounts like from about 0.5 to about 20 weight percent, and more specifically, from 1 to about 12 weight percent.

In various embodiments, the hole blocking layer further contains an optional light scattering particle. In various embodiments, the light scattering particle has a refractive index different from the resin mixture, and has a number average particle size greater than about 0.8 micron. The light scattering particle can be amorphous silica, and silicone ball. In various embodiments, the light scattering particle can be present in an amount of about 0 to about 10 percent by weight of a total weight of the hole blocking layer.

## PHOTOCONDUCTOR LAYER EXAMPLES

The thickness of the photoconductive substrate layer depends on many factors including economical considerations, electrical characteristics, and the like; thus, this layer may be of substantial thickness, for example over 3,000 microns, such as from about 500 to about 2,000 microns, from about 300 to about 700 microns, or of a minimum thickness. In embodiments, the thickness of this layer is from about 75 to about 300 microns, or from about 100 to about 150 microns.

The substrate may be opaque or substantially transparent, and may comprise any suitable material having the required mechanical properties. Accordingly, the substrate may comprise a layer of an electrically nonconductive or conductive material such as an inorganic or an organic composition. As electrically nonconducting materials, there may be employed various resins known for this purpose including polyesters, polycarbonates, polyamides, polyurethanes, and the like, which are flexible as thin webs. An electrically conducting substrate may be any suitable metal of, for example, aluminum, nickel, steel, copper, and the like, or a polymeric material, as described above, filled with an electrically conducting substance, such as carbon, metallic powder, and the like, or an organic electrically conducting material. The electrically insulating or conductive substrate may be in the form of an endless flexible belt, a web, a rigid cylinder, a sheet, and the like. The thickness of the substrate layer depends on numerous factors including strength desired and economical considerations. For a drum, as disclosed in a copending application referenced herein, this layer may be of a substantial thickness of, for example, up to many centimeters or of a minimum thickness of less than a millimeter. Similarly, a flexible belt may be of a substantial thickness of, for example, about 250 microns, or of minimum thickness of less than about 50 microns, provided there are no adverse effects on the final electrophotographic device. In embodiments where the substrate layer is not conductive, the surface thereof may be rendered electrically conductive by an electrically conductive coating. The conductive coating may vary in thickness over substantially wide ranges depending upon the optical transparency, degree of flexibility desired, and economic factors.

Illustrative examples of substrates are as illustrated herein, and more specifically, substrates selected for the imaging members of the present disclosure, and which substrates can be opaque or substantially transparent comprise a layer of insulating material including inorganic or organic polymeric materials, such as MYLAR® a commercially available polymer, MYLAR® containing titanium, a layer of an organic or inorganic material having a semiconductive surface layer, such as indium tin oxide, or aluminum arranged thereon, or a conductive material inclusive of aluminum, chromium,

## 12

nickel, brass, or the like. The substrate may be flexible, seamless, or rigid, and may have a number of many different configurations, such as for example, a plate, a cylindrical drum, a scroll, an endless flexible belt, and the like. In 5 embodiments, the substrate is in the form of a seamless flexible belt. In some situations, it may be desirable to coat on the back of the substrate, particularly when the substrate is a flexible organic polymeric material, an anticurl layer, such as for example polycarbonate materials commercially available 10 as MAKROLON®.

The photogenerating layer in embodiments is comprised of, for example, a number of known photogenerating pigments including, for example, Type V hydroxygallium phthalocyanine, Type IV or V titanyl phthalocyanine or chlorogallium phthalocyanine, and a resin binder like poly(vinyl chloride-co-vinyl acetate) copolymer, such as VMCH (available from Dow Chemical), or polycarbonate. Generally, the photogenerating layer can contain known photogenerating pigments, such as metal phthalocyanines, metal free phthalocyanines, alkylhydroxygallium phthalocyanines, hydroxygallium phthalocyanines, chlorogallium phthalocyanines, perylenes, especially bis(benzimidazo)perylene, titanyl phthalocyanines, and the like, and more specifically, vanadyl phthalocyanines, Type V hydroxygallium phthalocyanines, and inorganic components such as selenium, selenium alloys, and trigonal selenium. The photogenerating pigment can be dispersed in a resin binder similar to the resin binders selected for the charge transport layer, or alternatively no resin binder need be present. Generally, the thickness of the photogenerating layer depends on a number of factors, including the thicknesses of the other layers, and the amount of photogenerating material contained in the photogenerating layer. Accordingly, this layer can be of a thickness of, for example, from about 0.05 to about 10 microns, and more specifically, 15 from about 0.25 to about 2 microns when, for example, the photogenerating compositions are present in an amount of from about 30 to about 75 percent by volume. The maximum thickness of this layer in embodiments is dependent primarily 20 upon factors, such as photosensitivity, electrical properties and mechanical considerations. The photogenerating layer binder resin is present in various suitable amounts of, for example, from about 1 to about 50 weight percent, and more specifically, from about 1 to about 10 weight percent, and which resin may be selected from a number of known polymers, such as poly(vinyl butyral), poly(vinyl carbazole), 25 polyesters, polycarbonates, poly(vinyl chloride), polyacrylates and methacrylates, copolymers of vinyl chloride and vinyl acetate, phenolic resins, polyurethanes, poly(vinyl alcohol), polyacrylonitrile, polystyrene, and the like. It is desirable to select a coating solvent that does not substantially 30 disturb or adversely affect the other previously coated layers of the device. Generally, however, from about 5 to about 90 percent by volume of the photogenerating pigment is dispersed in about 10 to about 95 percent by volume of the resinous binder, or from about 20 to about 30 percent by volume of the photogenerating pigment is dispersed in about 35 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705

drofuran, dioxane, diethyl ether, dimethyl formamide, dimethyl acetamide, butyl acetate, ethyl acetate, methoxyethyl acetate, and the like.

The photogenerating layer may comprise amorphous films of selenium and alloys of selenium and arsenic, tellurium, germanium, and the like, hydrogenated amorphous silicone and compounds of silicone and germanium, carbon, oxygen, nitrogen, and the like fabricated by vacuum evaporation or deposition. The photogenerating layer may also comprise inorganic pigments of crystalline selenium and its alloys; Group II to VI compounds; and organic pigments such as quinacridones, polycyclic pigments such as dibromo anthranthrone pigments, perylene and perinone diamines, polynuclear aromatic quinones, azo pigments including bis-, tris- and tetrakis-azos, and the like dispersed in a film forming polymeric binder and fabricated by solvent coating techniques.

Examples of polymeric binder materials that can be selected as the matrix for the photogenerating layer components are thermoplastic and thermosetting resins, such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, poly(phenylene sulfides), poly(vinyl acetate), polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, poly(vinyl chloride), vinyl chloride and vinyl acetate copolymers, acrylate copolymers, alkyd resins, cellulosic film formers, poly(amideimide), styrene-butadiene copolymers, vinylidene chloride-vinyl chloride copolymers, vinyl acetate-vinylidene chloride copolymers, styrene-alkyd resins, poly(vinyl carbazole), and the like. These polymers may be block, random or alternating copolymers.

Various suitable and conventional known processes may be selected to mix, and thereafter apply the photogenerating layer coating mixture to the substrate, and more specifically, to the hole blocking layer or other layers like spraying, dip coating, roll coating, wire wound rod coating, vacuum sublimation, and the like. For some applications, the photogenerating layer may be fabricated in a dot or line pattern. Removal of the solvent of a solvent-coated layer may be effected by any known conventional techniques such as oven drying, infrared radiation drying, air drying, and the like. The coating of the photogenerating layer on the hole blocking layer in embodiments of the present disclosure can be accomplished such that the final dry thickness of the photogenerating layer is as illustrated herein, and can be, for example, from about 0.01 to about 30 microns after being dried at, for example, about 40 to about 150° C. for about 1 to about 90 minutes. More specifically, a photogenerating layer of a thickness, for example, of from about 0.1 to about 30 microns, or from about 0.5 to about 2 microns can be applied to or deposited on the substrate, on other surfaces in between the substrate and the charge transport layer, and the like. The hole blocking layer or undercoat layer (UCL) may be applied to the electrically conductive supporting substrate surface prior to the application of a photogenerating layer.

A suitable known adhesive layer can be included in the photoconductor. Typical adhesive layer materials include, for example, polyesters, polyurethanes, and the like. The adhesive layer thickness can vary, and in embodiments is, for example, from about 0.05 to about 0.3 micron. The adhesive layer can be deposited on the hole blocking layer by spraying, dip coating, roll coating, wire wound rod coating, gravure

coating, Bird applicator coating, and the like. Drying of the deposited coating may be effected by, for example, oven drying, infrared radiation drying, air drying, and the like. As optional adhesive layers usually in contact with or situated between the hole blocking layer and the photogenerating layer, there can be selected various known substances inclusive of copolyesters, polyamides, poly(vinyl butyral), poly(vinyl alcohol), polyurethane, and polyacrylonitrile. This layer is, for example, of a thickness of from about 0.001 to about 1 micron, or from about 0.1 to about 0.5 micron. Optionally, this layer may contain effective suitable amounts, for example from about 1 to about 10 weight percent, of conductive and nonconductive particles, such as zinc oxide, titanium dioxide, silicone nitride, carbon black, and the like, to provide, for example, in embodiments of the present disclosure, further desirable electrical and optical properties.

A number of charge transport materials, especially known hole transport molecules, may be selected for the charge transport layer, examples of which are aryl amines of the formulas/structures, and which layer is generally of a thickness of from about 5 to about 75 microns, and more specifically, of a thickness of from about 10 to about 40 microns



wherein X is a suitable hydrocarbon like alkyl, alkoxy, and aryl; a halogen, or mixtures thereof, and especially those substituents selected from the group consisting of Cl and CH<sub>3</sub>; and molecules of the following formulas



wherein X, Y and Z are a suitable substituent like a hydrocarbon, such as independently alkyl, alkoxy, or aryl; a halogen,

or mixtures thereof, and wherein at least one of Y or Z is present. Alkyl and alkoxy contain, for example, from 1 to about 25 carbon atoms, and more specifically, from 1 to about 12 carbon atoms, such as methyl, ethyl, propyl, butyl, pentyl, and the corresponding alkoxides. Aryl can contain from 6 to about 36 carbon atoms, such as phenyl, and the like. Halogen includes chloride, bromide, iodide, and fluoride. Substituted alkyls, alkoxy, and aryls can also be selected in embodiments. At least one charge transport refers, for example, to 1, from 1 to about 7, from 1 to about 4, and from 1 to about 2.

Examples of specific aryl amines include N,N'-diphenyl-N,N'-bis(alkylphenyl)-1,1'-biphenyl-4,4'-diamine wherein alkyl is selected from the group consisting of methyl, ethyl, propyl, butyl, hexyl, and the like; N,N'-diphenyl-N,N'-bis(halophenyl)-1,1'-biphenyl-4,4'-diamine wherein the halo substituent is a chloro substituent; N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis(4-isopropylphenyl)-[p-terphenyl]-4,4'-diamine, N,N'-bis(4-butylphenyl)-N,N'-bis(2-ethyl-6-methylphenyl)-[p-terphenyl]-4,4'-diamine, N,N'-bis(4-butylphenyl)-N,N'-bis(2,5-dimethylphenyl)-[p-terphenyl]-4,4'-diamine, N,N'-diphenyl-N,N'-bis(3-chlorophenyl)-[p-terphenyl]-4,4'-diamine, and the like. Other known charge transport layer molecules can be selected, reference for example, U.S. Pat. Nos. 4,921,773 and 4,464,450, the disclosures of which are totally incorporated herein by reference.

Examples of the binder materials selected for the charge transport layer or layers include components, such as those described in U.S. Pat. No. 3,121,006, the disclosure of which is totally incorporated herein by reference. Specific examples of polymer binder materials include polycarbonates, polyarylates, acrylate polymers, vinyl polymers, cellulose polymers, polyesters, polysiloxanes, polyamides, polyurethanes, poly(cyclo olefins), epoxies, and random or alternating copolymers thereof; and more specifically, polycarbonates such as poly(4,4'-isopropylidene-diphenylene)carbonate (also referred to as bisphenol-A-polycarbonate), poly(4,4'-cyclohexylidinediphenylene)carbonate (also referred to as bisphenol-Z-polycarbonate), poly(4,4'-isopropylidene-3,3'-dimethyl-diphenyl) carbonate (also referred to as bisphenol-C-polycarbonate), and the like. In embodiments, electrically inactive binders are comprised of polycarbonate resins with a molecular weight of from about 20,000 to about 100,000, or with a molecular weight  $M_w$  of from about 50,000 to about 100,000 preferred. Generally, the transport layer contains from about 10 to about 75 percent by weight of the charge transport material, and more specifically, from about 35 to about 50 percent of this material.

The charge transport layer or layers, and more specifically, a first charge transport in contact with the photogenerating layer, and thereover a top or second charge transport overcoating layer may comprise charge transporting small molecules dissolved or molecularly dispersed in a film forming electrically inert polymer such as a polycarbonate. In embodiments, "dissolved" refers, for example, to forming a solution in which the small molecule is dissolved in the polymer to form a homogeneous phase; and "molecularly dispersed in embodiments" refers, for example, to charge transporting molecules dispersed in the polymer, the small molecules being dispersed in the polymer on a molecular scale. Various charge transporting or electrically active small molecules may be selected for the charge transport layer or layers. In embodiments, charge transport refers, for example, to charge transporting molecules as a monomer that allows the free

charge generated in the photogenerating layer to be transported across the transport layer.

Examples of hole transporting molecules selected for the charge transport layer or layers, and present in various effective amounts, include, for example, pyrazolines such as 1-phenyl-3-(4'-diethylamino-styryl)-5-(4"-diethylamino phenyl)pyrazoline; aryl amines such as N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis(4-isopropylphenyl)-[p-terphenyl]-4,4'-diamine, N,N'-bis(4-butylphenyl)-N,N'-bis(2-ethyl-6-methylphenyl)-[p-terphenyl]-4,4'-diamine, N,N'-bis(4-butylphenyl)-N,N'-bis(2,5-dimethylphenyl)-[p-terphenyl]-4,4'-diamine, and N,N'-diphenyl-N,N'-bis(3-chlorophenyl)-[p-terphenyl]-4,4'-diamine; hydrazones such as N-phenyl-N-methyl-3-(9-ethyl) carbazyl hydrazone, and 4-diethyl amino benzaldehyde-1,2-diphenyl hydrazone; and oxadiazoles such as 2,5-bis(4-N,N'-diethylaminophenyl)-1,2,4-oxadiazole, stilbenes, and the like. A small molecule charge transporting compound that permits injection of holes into the photogenerating layer with high efficiency, and transports them across the charge transport layer with short transit times includes N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis(4-isopropylphenyl)-[p-terphenyl]-4,4'-diamine, N,N'-bis(4-butylphenyl)-N,N'-bis(2-ethyl-6-methylphenyl)-[p-terphenyl]-4,4'-diamine, N,N'-bis(4-butylphenyl)-N,N'-bis(2,5-dimethylphenyl)-[p-terphenyl]-4,4'-diamine, and N,N'-diphenyl-N,N'-bis(3-chlorophenyl)-[p-terphenyl]-4,4'-diamine, or mixtures thereof. If desired, the charge transport material in the charge transport layer may comprise a polymeric charge transport material or a combination of a small molecule charge transport material and a polymeric charge transport material.

Examples of components or materials optionally incorporated into the charge transport layers or at least one charge transport layer to, for example, enable improved lateral charge migration (LCM) resistance include hindered phenolic antioxidants, such as tetrakis methylene(3,5-di-tert-butyl-4-hydroxy hydrocinnamate)methane (IRGANOX<sup>TM</sup> 1010, available from Ciba Specialty Chemical), butylated hydroxytoluene (BHT), and other hindered phenolic antioxidants including SUMILIZER<sup>TM</sup> BHT-R, MDP-S, BBM-S, WX-R, NW, BP-76, BP-101, GA-80, GM and GS (available from Sumitomo Chemical Co., Ltd.), IRGANOX<sup>TM</sup> 1035, 1076, 1098, 1135, 1141, 1222, 1330, 1425WL, 1520L, 245, 259, 3114, 3790, 5057 and 565 (available from Ciba Specialties Chemicals), and ADEKA STAB<sup>TM</sup> AO-20, AO-30, 55 AO-40, AO-50, AO-60, AO-70, AO-80 and AO-330 (available from Asahi Denka Co., Ltd.); hindered amine antioxidants such as SANOL<sup>TM</sup> LS-2626, LS-765, LS-770 and LS-744 (available from SNKYO CO., Ltd.), TINUVINT<sup>TM</sup> 144 and 622LD (available from Ciba Specialties Chemicals), MARK<sup>TM</sup> LA57, LA67, LA62, LA68 and LA63 (available from Asahi Denka Co., Ltd.), and SUMILIZER<sup>TM</sup> TPS (available from Sumitomo Chemical Co., Ltd.); thioether antioxidants such as SUMILIZER<sup>TM</sup> TP-D (available from Sumitomo Chemical Co., Ltd.); phosphite antioxidants such as MARK<sup>TM</sup> 2112, PEP-8, PEP-24G, PEP-36, 329K and HP-10 (available from Asahi Denka Co., Ltd.); other molecules such as bis(4-diethylamino-2-methylphenyl)phenylmethane

17

(BDETPM), bis-[2-methyl-4-(N-2-hydroxyethyl-N-ethyl-aminophenyl)]-phenylmethane (DHTPM), and the like. The weight percent of the antioxidant in at least one of the charge transport layers is from about 0 to about 20 weight percent, from about 1 to about 10 weight percent, or from about 3 to about 8 weight percent.

A number of processes may be used to mix, and thereafter apply the charge transport layer or layers coating mixture to the photogenerating layer. Typical application techniques include spraying, dip coating, and roll coating, wire wound rod coating, and the like. Drying of the charge transport deposited coating may be effected by any suitable conventional technique such as oven drying, infrared radiation drying, air drying, and the like.

The thickness of each of the charge transport layers in embodiments is, for example, from about 10 to about 75 microns, from about 15 to about 50 microns, but thicknesses outside these ranges may in embodiments also be selected. The charge transport layer should be an insulator to the extent that an electrostatic charge placed on the hole transport layer is not conducted in the absence of illumination at a rate sufficient to prevent formation and retention of an electrostatic latent image thereon. In general, the ratio of the thickness of the charge transport layer to the photogenerating layer can be from about 2:1 to about 200:1, and in some instances 400:1. The charge transport layer is substantially nonabsorbing to visible light or radiation in the region of intended use, but is electrically "active" in that it allows the injection of photogenerated holes from the photoconductive layer or photogenerating layer, and allows these holes to be transported through itself to selectively discharge a surface charge on the surface of the active layer.

The thickness of the continuous charge transport layer selected depends upon the abrasiveness of the charging (bias charging roll), cleaning (blade or web), development (brush), transfer (bias transfer roll), and the like in the system employed, and can be up to about 10 microns. In embodiments, the thickness for each charge transport layer can be, for example, from about 1 to about 5 microns. Various suitable and conventional methods may be used to mix, and thereafter apply an overcoat top charge transport layer coating mixture to the photoconductor. Typical application techniques include spraying, dip coating, roll coating, wire wound rod coating, and the like. Drying of the deposited coating may be effected by any suitable conventional technique, such as oven drying, infrared radiation drying, air drying, and the like. The dried overcoating layer of this disclosure should transport holes during imaging, and should not have too high a free carrier concentration. Free carrier concentration in the overcoat increases the dark decay.

The following Examples are provided. All proportions are by weight unless otherwise indicated.

#### COMPARATIVE EXAMPLE 1

A dispersion of a hole blocking layer was prepared by milling 18 grams of  $\text{TiO}_2$  (MT-150W, manufactured by Tayca Co., Japan), 24 grams of the phenolic resin (VARCUM® 29159, OxyChem Co., about 50 percent in xylene/1-butanol=50/50) at a solid weight ratio of about 60 to about 40 in a solvent mixture of xylene and 1-butanol (50/50 mixture), and a total solid content of about 48 percent in an attritor mill with about 0.4 to about 0.6 millimeter size  $\text{ZrO}_2$  beads for 6.5 hours, and then filtering with a 20 micron Nylon filter. A 30 millimeter aluminum drum substrate was then coated with the aforementioned generated dispersion using known coating techniques as illustrated herein. After drying at 160° C. for 20

18

minutes, a hole blocking layer of  $\text{TiO}_2$  in the phenolic resin ( $\text{TiO}_2$ /phenolic resin=60/40) about 15 microns in thickness was obtained.

A photogenerating layer comprising chlorogallium phthalocyanine (Type C) was deposited on the above hole blocking layer or undercoat layer at a thickness of about 0.2 micron. The photogenerating layer coating dispersion was prepared as follows. 2.7 Grams of chlorogallium phthalocyanine (Cl-GaPc) Type C pigment were mixed with 2.3 grams of the polymeric binder (carboxyl modified vinyl copolymer, VMCH, Dow Chemical Company), 15 grams of n-butyl acetate, and 30 grams of xylene. The resulting mixture was milled in an attritor mill with about 200 grams of 1 millimeter Hi-Bea borosilicate glass beads for about 3 hours. The dispersion mixture obtained was then filtered through a 20 micron Nylon cloth filter, and the solids content of the dispersion was diluted to about 6 weight percent.

Subsequently, a 29 micron (A) or 15 micron (B) charge transport layer was coated on top of the photogenerating layer from a dispersion prepared from N,N'-diphenyl-N,N'-bis(3-methylphenyl)-1,1'-biphenyl-4,4'-diamine (5.38 grams), a film forming polymer binder, PCZ-400 [poly(4,4'-dihydroxydiphenyl-1-1-cyclohexane,  $M_w$ =40,000)] available from Mitsubishi Gas Chemical Company, Ltd. (7.13 grams), and PTFE POLYFLONTM L-2 microparticle (1 gram), available from Daikin Industries, dissolved/dispersed in a solvent mixture of 20 grams of tetrahydrofuran (THF), and 6.7 grams of toluene through a CAVIPRO™ 300 nanomizer (Five Star Technology, Cleveland, Ohio). The charge transport layer was dried at about 120° C. for about 40 minutes.

#### EXAMPLE I

Two photoconductors (A) and (B) were prepared by repeating the process of Comparative Example 1 (A) and 1 (B), respectively, except that the hole blocking layer dispersion was prepared by milling 19.5 grams of  $\text{TiO}_2$  (MT-150W, manufactured by Tayca Co., Japan), 7 grams of the epoxy resin (EPON™ 1001-T-75, 450 to 550 weight per epoxide, 75 percent solids in toluene, obtained from Hexion Specialty Chemicals), and 9.46 grams of the carboxyl resin (PARALOID® AT-81,  $T_g$ =40° C., acid number=65, 55.5 percent solid in the aromatic solvent 150/butyl cellulose=87/13, obtained from Rohm and Haas) at a solid weight ratio of about 65 to about 17.5 to about 17.5 in a solvent mixture of xylene and 1-butanol (50/50 mixture), and a total solid content of about 45 percent in an attritor mill with about 0.4 to about 0.6 millimeter size  $\text{ZrO}_2$  beads for 6.5 hours, and then filtering with a 20 micron Nylon filter. The resulting dispersion was then added to 0.3 gram of the base catalyst, triethylamine, and mixed for an hour. A 30 millimeter aluminum drum substrate was then coated with the aforementioned generated dispersion using known coating techniques as illustrated herein. After drying at 180° C. for 20 minutes, a hole blocking layer of  $\text{TiO}_2$  in the crosslinked epoxy/carboxyl resin mixture ( $\text{TiO}_2$ /epoxy resin/carboxyl resin=65/17.5/17.5) about 15 microns in thickness was obtained.

#### EXAMPLE II

Two photoconductors (A) and (B) were prepared by repeating the process of Example I (A) and I (B), respectively, except that the hole blocking layer was dried at 200° C. for 20 minutes.

#### EXAMPLE III

Two photoconductors (A) and (B) were prepared by repeating the process of Comparative Example 1 (A) and 1 (B),

respectively, except that the hole blocking layer dispersion was prepared by milling 19.5 grams of  $\text{TiO}_2$  (MT-150W, manufactured by Tayca Co., Japan), 4.2 grams of the epoxy resin (EPON<sup>TM</sup> 1001-T-75, 450 to 550 weight per epoxide, 75 percent solids in toluene, obtained from Hexion Specialty Chemicals), and 13.24 grams of the carboxyl resin (PARALOID<sup>®</sup> AT-81,  $T_g=40^\circ\text{C}$ ., acid number=65, 55.5 percent solid in the aromatic solvent 150/butyl cellosolve=87/13, obtained from Rohm and Haas) at a solid weight ratio of about 65 to about 10.5 to about 24.5 in a solvent mixture of xylene and 1-butanol (50/50 mixture), and a total solid content of about 45 percent in an attritor mill with about 0.4 to about 0.6 millimeter size  $\text{ZrO}_2$  beads for 6.5 hours, and then filtering with a 20 micron Nylon filter. The dispersion was then added with 0.3 gram of the base catalyst, triethylamine, and mixed for an hour. A 30 millimeter aluminum drum substrate was then coated with the aforementioned generated dispersion using known coating techniques as illustrated herein. After drying at  $180^\circ\text{C}$ . for 20 minutes, a hole blocking layer of  $\text{TiO}_2$  in the epoxy/carboxyl resin mixture ( $\text{TiO}_2$ /epoxy resin/carboxyl resin=65/10.5/24.5) about 15 microns in thickness was obtained.

#### EXAMPLE IV

Two photoconductors (A) and (B) were prepared by repeating the process of Example III (A) and III (B), respectively, except that the hole blocking layer was dried at  $200^\circ\text{C}$ . for 20 minutes.

#### ELECTRICAL PROPERTY TESTING

The above prepared photoconductors of Comparative Example 1 (A) and Examples I (A), II (A), III (A) and IV (A) were tested in a scanner set to obtain photoinduced discharge cycles, sequenced at one charge-erase cycle followed by one charge-expose-erase cycle, wherein the light intensity was incrementally increased with cycling to produce a series of photoinduced discharge characteristic (PIDC) curves from which the photosensitivity and surface potentials at various exposure intensities were measured. Additional electrical characteristics were obtained by a series of charge-erase cycles with incrementing surface potential to generate several voltages versus charge density curves. The scanner was equipped with a scorotron set to a constant voltage charging at various surface potentials. These two photoconductors were tested at surface potentials of 700 volts with the exposure light intensity incrementally increased by regulating a series of neutral density filters; the exposure light source is a 780 nanometer light emitting diode. The xerographic simulation was completed in an environmentally controlled light tight chamber at ambient conditions (40 percent relative humidity and  $22^\circ\text{C}$ .).

The  $V_r$  (residual potential after erase) was used to characterize the photoconductors with the results being shown in Table 1. The disclosed photoconductors of Examples I (A), II (A), III (A) and IV (A) exhibited about 30 to about 50 volts lower  $V_r$  than the photoconductor of Comparative Example 1 (A).

TABLE 1

| Photoconductors           | $V_r$ (V) |
|---------------------------|-----------|
| Comparative Example 1 (A) | 116       |
| Example I (A)             | 101       |
| Example II (A)            | 124       |

TABLE 1-continued

| Photoconductors | $V_r$ (V) |
|-----------------|-----------|
| Example III (A) | 124       |
| Example IV (A)  | 150       |

#### GHOSTING MEASUREMENT

The Comparative Example 1 (A) and Examples I (A), II (A), III (A) and IV (A) photoconductors were acclimated at room temperature for 24 hours before testing in A zone ( $85^\circ\text{F}$ . and 80 percent humidity) for ghosting. Print testing was accomplished in the Xerox Corporation WorkCentre<sup>TM</sup> Pro C3545 using the K (black toner) station at  $t$  of 500 print counts ( $t$  equal to 0 is the first print;  $t$  equal to 500 is the 500<sup>th</sup> print). At the CMY stations of the color WorkCentre<sup>TM</sup> Pro C3545, run-up from  $t$  of 0 to  $t$  of 500 print counts for the photoconductor was completed. The prints for determining ghosting characteristics includes an X symbol or letter on a half tone image. When X is visible, the ghost level is assigned Grade 0; when X is barely visible, the ghost level is assigned Grade 1; Grade 2 to Grade 5 refers to the level of visibility of X with Grade 5 meaning a dark and visible X. Ghosting levels were visually measured against an empirical scale, the smaller the ghosting grade (absolute value), the better the print quality. The ghosting results are summarized in Table 2.

TABLE 2

| Photoconductors           | Ghosting Grade at $t$ of 0 | Ghosting at $t$ of 500 prints |
|---------------------------|----------------------------|-------------------------------|
| Comparative Example 1 (A) | Grade -3                   | Grade -5                      |
| Example I (A)             | Grade 0                    | Grade -1                      |
| Example II (A)            | Grade 0                    | Grade -1.5                    |
| Example III (A)           | Grade -1                   | Grade -1.5                    |
| Example IV (A)            | Grade -1                   | Grade -1.5                    |

After 500 prints, the ghosting level for the Example photoconductors remained low at Grade -1 to -1.5; in contrast, the Comparative Example 1 (A) photoconductor had an elevated ghosting level of Grade -5. The disclosed hole blocking layer comprised of the epoxy/carboxyl resin mixture exhibited almost no ghosting; in contrast, the Comparative hole blocking layer comprised of the phenolic resin exhibited high ghosting.

#### BACKGROUND/CHARGE DEFICIENT SPOT MEASUREMENT

The Comparative Example 1 (B) and Examples I (B), II (B), III (B) and IV (B) photoconductors were acclimated at room temperature for 24 hours before testing in A zone ( $85^\circ\text{F}$ /80 percent relative humidity) for background/charge deficient spot (CDS). Print testing was completed in the Xerox Corporation WorkCentre<sup>TM</sup> Pro C3545 using the black and white copy mode, and where there was achieved a machine speed of 165 millimeters/second at  $t$  equal to 0 for background/CDS. Background/CDS levels were visually measured against an empirical scale where the smaller the background/CDS grade level, the better the print quality. The results are shown in Table 3. More specifically, background/CDS is a measure of the percentage of grayness on white paper; Grade 1, on this scale, is almost white, while Grade 2 represents unacceptable dark prints.

## 21

TABLE 3

| Photoconductors           | Background/CDS Grade |
|---------------------------|----------------------|
| Comparative Example 1 (A) | Grade 2              |
| Example I (A)             | Grade 1              |
| Example II (A)            | Grade 1              |
| Example III (A)           | Grade 1              |
| Example IV (A)            | Grade 1              |

The photoconductors that contain the disclosed hole blocking layer comprised of the epoxy/carboxyl resin mixture exhibited almost no background/CDS, while in contrast, the Comparative hole blocking layer comprised of the phenolic resin exhibited 100 percent higher background/CDS.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others. Unless specifically recited in a claim, steps or components of claims should not be implied or imported from the specification or any other claims as to any particular order, number, position, size, shape, angle, color, or material.

## What is claimed is:

1. A photoconductor consisting of a substrate; an undercoat layer thereover wherein the undercoat layer consists of a metal oxide, and a mixture that consists of an epoxy resin and a carboxyl resin; a photogenerating layer; and at least one aryl amine charge transport layer; and wherein said epoxy resin possesses a weight average molecular weight of from about 60 to about 30,000, and said carboxyl resin possesses a weight average molecular weight of from about 500 to about 100,000 and wherein said resin mixture is present in an amount of from about 20 to about 60 weight percent, and wherein the total of said components in said undercoat layer is about 100 percent; wherein said mixture of the epoxy resin and the carboxyl resin is crosslinked by the use of a catalyst.

2. A photoconductor in accordance with claim 1 wherein said metal oxide is a titanium oxide.

3. A photoconductor in accordance with claim 1 wherein said metal oxide is present in an amount of from about 20 percent to about 80 percent by weight of the total weight of the undercoat layer components.

4. A photoconductor in accordance with claim 1 wherein said resin mixture is present in said undercoat layer in an amount of from about 20 to about 50 weight percent.

5. A photoconductor in accordance with claim 1 wherein said epoxy resin is present in said resin mixture in an amount of from about 1 to about 99 weight percent, and said carboxyl resin is present in said resin mixture in an amount of from about 99 to about 1 weight percent, and wherein the total resin mixture thereof is about 100 percent.

6. A photoconductor in accordance with claim 1 wherein said epoxy resin is selected from the group consisting of diglycidyl ether of bisphenol A epoxy resin, diglycidyl ether of bisphenol F epoxy resin, tetraglycidyl ether of tetraphenol ethane epoxy resin, epoxy phenolic novolac resin, epoxy bisphenol A novolac resin, epoxy bisphenol F novolac resin, epoxy cresol novolac resin, epoxy polyacrylate, elastomer modified epoxy resin, hydrogenated diglycidyl ether of bisphenol A epoxy resin, cycloaliphatic glycidyl ether epoxy resin, brominated epoxy, alkyl glycidyl ether epoxy resin, cresyl glycidyl ether epoxy resin, butyl glycidyl ether epoxy resin, castor oil glycidyl ether epoxy resin, and optionally mixtures thereof.

## 22

7. A photoconductor in accordance with claim 1 wherein said epoxy resin is a diglycidyl ether of bisphenol A epoxy resin and a diglycidyl ether of bisphenol F epoxy resin, and mixtures thereof.

8. A photoconductor in accordance with claim 1 wherein said crosslinking is from about 60 to about 95 percent.

9. A photoconductor in accordance with claim 1 wherein said catalyst is an acid selected from a group consisting of oxalic acid, maleic acid, carboxylic acid, ascorbic acid, malonic acid, succinic acid, tartaric acid, citric acid, p-toluenesulfonic acid, methanesulfonic acid, and mixtures thereof, present in an amount of from about 0.1 to about 5 weight percent based on the total weight of said resin mixture; or a base selected from a group consisting of triethyl amine, diethylenetriamine, triethylenetetramine, isphoronediamine, bis-p-aminocyclohexylmethane, 1,2-diaminocyclohexane, diaminodiphenylmethane, and mixtures thereof, present in an amount of from about 0.1 to about 10 weight percent based on the total weight of said resin mixture.

10. A photoconductor in accordance with claim 1 wherein said metal oxide is present in an amount of from about 50 percent to about 70 percent based on the total weight of the undercoat layer components.

11. A photoconductor in accordance with claim 1 wherein said metal oxide possesses a size diameter of from about 5 to about 300 nanometers, and a powder resistivity of from about  $1 \times 10^3$  to about  $1 \times 10^8$  ohm/cm when applied at a pressure of from about 50 to about 650 kilograms/cm<sup>2</sup>.

12. A photoconductor in accordance with claim 1 wherein said metal oxide is surface treated with aluminum laurate, alumina, zirconia, silica, silane, methicone, dimethicone, sodium metaphosphate or mixtures thereof.

13. A photoconductor in accordance with claim 1 wherein said metal oxide is a titanium oxide surface treated with an alkali metaphosphate.

14. A photoconductor in accordance with claim 1 wherein the thickness of the undercoat layer is from about 0.1 micron to about 30 microns.

15. A photoconductor in accordance with claim 1 wherein the thickness of the undercoat layer is from about 1 micron to about 15 microns, and said metal oxide is titanium oxide, zinc oxide or tin oxide.

16. A photoconductor in accordance with claim 1 wherein said charge transport layer is comprised of at least one of



wherein X is selected from the group consisting of alkyl, alkoxy, aryl, and halogen, and mixtures thereof.

17. A photoconductor in accordance with claim 1 wherein said charge transport layer consists of at least one of



wherein X, Y, and Z are independently selected from the group consisting of alkyl, alkoxy, aryl, and halogen, and mixtures thereof; wherein said epoxy resin is selected from the group consisting of diglycidyl ether of bisphenol A epoxy resin, diglycidyl ether of bisphenol F epoxy resin, tetraglycidyl ether of tetraphenol ethane epoxy resin, epoxy phenolic novolac resin, epoxy bisphenol A novolac resin, epoxy bisphenol F novolac resin, epoxy cresol novolac resin, epoxy polyacrylate, elastomer modified epoxy resin, hydrogenated diglycidyl ether of bisphenol A epoxy resin, cycloaliphatic glycidyl ether epoxy resin, brominated epoxy, alkyl glycidyl ether epoxy resin, cresyl glycidyl ether epoxy resin, butyl glycidyl ether epoxy resin, castor oil glycidyl ether epoxy resin, and optionally mixtures thereof; and wherein said carboxyl resin is an acrylic carboxyl resin polymerized from acrylic acid, methacrylic acid, and their derivatives, and mixtures thereof.

**18.** A photoconductor in accordance with claim 1 wherein said charge transport layer is comprised of a component selected from the group consisting of N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis-(4-isopropylphenyl)-[p-terphenyl]-4,4'-diamine, N,N'-bis(4-butylphenyl)-N,N'-bis-(2-ethyl-6-methylphenyl)-[p-terphenyl]-4,4'-diamine, N,N'-bis(4-butylphenyl)-N,N'-bis-(2,5-dimethylphenyl)-[p-terphenyl]-4,4'-diamine, and N,N'-diphenyl-N,N'-bis(3-chlorophenyl)-[p-terphenyl]-4,4'-diamine.

**19.** A photoconductor in accordance with claim 1 wherein said photogenerating layer is comprised of at least one photogenerating pigment.

**20.** A photoconductor in accordance with claim 19 wherein said photogenerating pigment is comprised of at least one of a titanyl phthalocyanine, a hydroxygallium phthalocyanine, a halogallium phthalocyanine, and mixtures thereof.

**21.** A photoconductor in accordance with claim 1 wherein said at least one charge transport layer is from 1 to about 4 layers.

**22.** A photoconductor in accordance with claim 1 wherein said at least one charge transport layer consists of a charge transport component and a resin binder; wherein said photogenerating layer consists of at least one photogenerating pig-

ment and a resin binder; and wherein said photogenerating layer is situated between said substrate and said charge transport layer, and wherein said epoxy resin possesses a weight average molecular weight of from about 500 to about 3,000, and said carboxyl resin possesses a weight average molecular weight of from about 1,500 to about 20,000.

**23.** A photoconductor consisting of a substrate; an undercoat layer thereover consisting of a mixture consisting of a metal oxide, and a crosslinked mixture of a crosslinked epoxy resin and a carboxyl resin; a photogenerating layer; and a charge transport layer, wherein said resin mixture is present in an amount of from about 20 to about 60 weight percent, wherein the total of said components in said undercoat layer is about 100 percent, wherein said epoxy resin is present in said resin mixture in an amount of from about 10 to about 40 weight percent, and said carboxyl resin is present in said resin mixture in an amount of from about 90 to about 60 weight percent, and wherein the total resin mixture solids thereof is about 100 percent; and wherein said epoxy resin possesses a weight average molecular weight of from about 250 to about 12,000, and said carboxyl resin possesses a weight average molecular weight of from about 1,500 to about 20,000.

**24.** A rigid or flexible photoconductor consisting of in sequence a supporting substrate; a hole blocking layer of a titanium oxide, and a mixture consisting of an epoxy resin and a carboxyl resin; a photogenerating layer, and a charge transport layer; and wherein the mixture is crosslinked at a percentage of from about 60 to about 95 percent, and which crosslinking is accomplished with a catalyst, and wherein said epoxy resin is a diglycidyl ether of bisphenol A epoxy resin, a diglycidyl ether of bisphenol F epoxy resin, and mixtures thereof; wherein said catalyst is an acid selected from a group consisting of oxalic acid, maleic acid, carboxylic acid, ascorbic acid, malonic acid, succinic acid, tartaric acid, citric acid, p-toluenesulfonic acid, methanesulfonic acid, and mixtures thereof, present in an amount of from about 0.1 to about 5 weight percent based on the total weight of said resin mixture; or a base selected from a group consisting of triethyl amine, diethylenetriamine, triethylenetetraamine, isphoronediamine, bis-p-aminocyclo hexylmethane, 1,2-diaminocyclohexane, diaminodiphenylmethane, and mixtures thereof, present in an amount of from about 0.1 to about 10 weight percent based on the total weight of said resin mixture, and wherein said carboxyl resin is an acrylic carboxyl resin and wherein said epoxy resin possesses a weight average molecular weight of from about 60 to about 30,000, and said carboxyl resin possesses a weight average molecular weight of from about 1,500 to about 20,000.

**25.** A photoconductor in accordance with claim 23 wherein said epoxy resin is selected from the group consisting of diglycidyl ether of bisphenol A epoxy resin, diglycidyl ether of bisphenol F epoxy resin, tetraglycidyl ether of tetraphenol ethane epoxy resin, epoxy phenolic novolac resin, epoxy bisphenol A novolac resin, epoxy bisphenol F novolac resin, epoxy cresol novolac resin, epoxy polyacrylate, elastomer modified epoxy resin, hydrogenated diglycidyl ether of bisphenol A epoxy resin, cycloaliphatic glycidyl ether epoxy resin, brominated epoxy, alkyl glycidyl ether epoxy resin, cresyl glycidyl ether epoxy resin, butyl glycidyl ether epoxy resin, and castor oil glycidyl ether epoxy resin.